

# UNITED STATES PATENT OFFICE.

HAROLD HIBBERT, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## EXPLOSIVE.

994,842.

Specification of Letters Patent. Patented June 13, 1911.

No Drawing.

Application filed September 15, 1910. Serial No. 582,145.

To all whom it may concern:

Be it known that I, HAROLD HIBBERT, a subject of the King of Great Britain, residing at Wilmington, county of Newcastle, 5 and State of Delaware, have invented a new and useful Improvement in Explosives, of which the following is a full, clear, and exact description.

When glycerin is treated with the mixed 10 acids, nitric acid and sulfuric acid, for the production of glycerin trinitrate, glycerin trinitrate is produced, the formula of which is:



This glycerin trinitrate has certain defects, among which it may be stated that 20 the glycerin which is its base is expensive, and the temperature of explosion of the explosive mixture of the glycerin trinitrate is very high, which makes it in many cases not a good ingredient for smokeless powder. 25 I have discovered that if nitrated butylene glycol be formed, a product is obtained whose temperature of explosive ignition is lower than that of glycerin trinitrate, which enables it to be freely used as an ingredient 30 of smokeless powder, safety explosives and dynamite. Further, I have discovered that such compound may be combined with nitrated derivatives, such, for instance, as nitrated cellulose or nitrated starch, to form 35 a colloid of such mixtures. It also may be mixed with glycerin trinitrate, and the resulting mixture has a lower freezing point and is more stable than glycerin trinitrate.

While butylene glycol is known and is 40 described in text books, I believe myself to be the first to have discovered nitrated butylene glycol and its value for the purposes named. Further, the method of making butylene glycol, as set out in the text 45 books, is so complicated as to render it very expensive and difficult to carry out. My discovery, therefore, includes a simple method for directly producing this butylene glycol as well as the nitrated butylene 50 glycol.

The butylene glycol is represented in formula in the following manner:



and when nitrated the formula is thus represented:



I produce the butylene glycol in the following manner: I take ethyl alcohol ( $\text{C}_2\text{H}_5\text{OH}$ ), which may be de-natured without affecting the result. This ethyl alcohol is first oxidized. Preferably I accomplish this oxidation by the ordinary catalytic oxidation, such for instance, by using metallic platinum, copper or zinc and heat. The resultant is acetaldehyde ( $\text{C}_2\text{H}_4\text{O}$ ). This acetaldehyde is then condensed. I have used for this condensation an aqueous solution of an alkaline carbonate, for instance, potassium carbonate; 450 grams of acetaldehyde were 65 cooled to  $-5^\circ \text{ C}$ . and 200 grams of powdered ice then added. A few drops of a cooled solution of potassium carbonate containing 19 grams of the carbonate in 60 cubic centimeters of water were introduced 70 into this mixture, the temperature not being allowed to rise above  $+10^\circ \text{ C}$ . After standing some 10 or 15 minutes a further quantity of the carbonate solution was introduced 75 and again allowed to stand, contents 80 being kept as nearly as possible at a temperature of  $0^\circ \text{ C}$ . After the whole of the carbonate had been added, the reaction-product was kept in ice-water for several 85 hours to prevent any rise of temperature 90 and then for a further 20 hours at  $+8$  to  $+10^\circ \text{ C}$ . If the pure acetaldol is required this may be extracted with ether, but for the purpose of obtaining butylene glycol this is unnecessary. The condensation can be produced by other alkaline carbonate of a borate, phosphate, acetate or cyanid, of the alkaline metals or alkaline earths. The resultant of this condensation is acetaldol 95 ( $\text{C}_4\text{H}_8\text{O}_2$ ). This condensation product is 100

then reduced to butylene glycol by means of a reducing agent, and I have employed the following method: The aqueous solution of acetaladol, obtained by condensing 450 grams of acetaldehyde with potassium carbonate was diluted to six liters with ice-water, rendered neutral by the addition of hydrochloric acid and then 142 grams of aluminum amalgam added. After standing for 10 two days, the aluminum hydroxid was filtered off and a further 58 grams of the amalgam added, and the mixture left for a further two days. After filtering the solution, the butylene glycol was recovered by 15 evaporating off the water under reduced pressure. Other amalgams may be used, and, further, the aluminum or other metal or an alloy or several metals may be used and also without the use of mercury. In 20 this condition the butylene glycol exists in an aqueous solution and is isolated by simple distillation, preferably under vacuum. This butylene glycol may then be nitrated in the same manner that glycerin is nitrated, by 25 means of nitric acid and sulfuric acid, in the following manner: 350 grams of ordinary nitrating acid such as is used for the nitration of glycerin were cooled to  $-5^{\circ}$  C. and then 50 grams of butylene glycol slowly 30 introduced into this, under the surface of the liquid in a fine spray, the acid being kept at  $-5^{\circ}$  C. and agitated vigorously throughout the addition. The butylene glycol dinitrate at once rises to the surface as a yellow oil and may be separated without further difficulty from the acid mixture. The resultant nitrated compound may then be 35 used by itself or mixed with a nitrate or nitrates, such as nitrated cellulose or nitrated starch. Indeed, I have found it quite valuable when mixed with glycerin trinitrate, as it then lowers the freezing point of glycerin trinitrate. Butylene glycol dinitrate may also be mixed with a nitro compound 40

or nitro compounds, as, for instance, tetra-nitro-methane, tri-nitro-toluene, nitro-naphthalene, or tri-nitro-anisol. Examples of such mixtures which may be used, are 80 parts by weight of butylene glycol nitrate and 20 parts by weight of tetra-nitro-methane, or 3 parts by weight of butylene glycol nitrate, 1 part by weight of tri-nitro-toluene and 1 part by weight of nitro-naphthalene. 45 50

When I speak of glycerin trinitrate, of course I intend to include the glycerin mono- and di-nitrates, although I have shown only the formula of the glycerin trinitrate. In like manner, when I use the term nitrated butylene glycol I intend to include the butylene glycol mono-nitrate and the butylene glycol dinitrate, although I have only shown the formula of the butylene glycol dinitrate. 55 60

I do not claim herein either the butylene glycol nitrate alone or mixed with a nitrate or nitrates as the same forms the subject matter of the claims of an application filed by me June 15th, 1910, Serial No. 566,934. Nor do I claim herein the method of producing butylene glycol, herein described, as 65 that is claimed in an application filed by me September 15th, 1910, Serial No. 582,144. 70

Having now fully described my invention, what I claim and desire to protect by Letters Patent is: 75

1. An explosive containing an admixture of butylene glycol nitrate and a nitro compound.
2. An explosive containing an admixture of butylene glycol nitrate and nitro compounds. 80

In testimony of which invention, I have hereunto set my hand, at Wilmington, Del. on this 10th day of Sept., 1910.

HAROLD HIBBERT.

Witnesses:

J. ED. WILSON,  
J. A. CASEY.

---

Copies of this patent may be obtained for five cents each, by addressing the "Commissioner of Patents, Washington, D. C."

---